

# UNITED STATES PATENT OFFICE.

SAMUEL CLELAND DAVIDSON, OF BELFAST, IRELAND.

## PEAT FUEL.

1,384,012.

Specification of Letters Patent. Patented July 5, 1921.

No Drawing.

Application filed February 7, 1920. Serial No. 357,928.

To all whom it may concern:

Be it known that I, SAMUEL CLELAND DAVIDSON, a subject of the King of Great Britain and Ireland, of Sirocco Engineering Works, Belfast, Ireland, merchant, have invented certain new and useful Improvements in the Preparation of Peat Fuel, of which the following is a specification.

My herein described improvements relate 10 to the preparation of a special type of peat fuel for employment in closed or open fire-grates, as a substitute for coal for general and household purposes, and the object of my invention is to economically produce this 15 class of peat fuel in large quantities by a commercially operative method.

In carrying my invention into effect, according to one modification, I take a suitable quantity of ordinary wet peat as obtained 20 directly from the bog, and work it in any suitable form of mixing machine (such, for example, as a dough-mixing machine) until it attains a putty-like consistency, and while continuing this mixing 25 process, add gradually thereto, and thoroughly blend therewith, stable proportions of powdered pitch, and of powdered dry peat. The latter can be easily and quickly made by passing common air-dried peat 30 through a power-driven centrifugally-acting disintegrating machine, which almost instantaneously reduces it to the powdered condition which I herein refer to as "powdered dry peat." The proportions may 35 vary, but enough pitch is used to give a luminous bituminous flame, which requires not to exceed one-half the weight of the wet peat. Of the dry powdered peat enough is used to give a suitably coherent product 40 having no apparent excess of moisture, which requires not to exceed two-thirds the weight of the wet peat.

The blending together of these three materials is then continued until the mixture 45 attains the condition of one homogeneous mass, from which suitable quantities can be taken and pressed in molds into blocks, during which operation but little fluid exudes therefrom, even with an applied pressure 50 sure up to as much as half a ton to the square inch.

The pressed blocks should be allowed to mature for a few days under cover from the weather, as maturing in this way toughens 55 and hardens them, and also causes them to ignite more readily in either open or closed

fire-grates, and to burn, firstly, with a bright yellow flame, and in the subsequent incandescent stage with substantially an equal durability to that of good quality 60 bituminous coal, so that although their calorific value is lower than that of coal, they can nevertheless be satisfactorily employed as a substitute therefor, more especially when used in open fire-grates for 65 household purposes.

The relative proportions of the several component materials used in the manufacture of the herein described peat fuel, may be varied within wide limits according to 70 the quality and condition of the wet peat as obtained from the bog and of the powdered dry peat, the object in view throughout being to so adjust these relative proportions, consistently with the maintenance of 75 good combustion, that when the whole mixture is blended into a homogeneous mass, and suitable quantities from it are being pressed into blocks, very little fluid will exude therefrom, so that without further treatment, beyond allowing the blocks to mature for a few days under cover from the weather, they will toughen and harden into a good general and household fuel, which will burn satisfactorily in open or closed 80 fire-grates, and constitute a useful substitute for coal.

I have operated with satisfactory results, using from  $\frac{1}{8}$  to  $\frac{1}{2}$  of the weight of the wet peat of pitch, and from  $\frac{1}{6}$  to  $\frac{1}{3}$  of such weight 90 of dry peat.

I do not herein claim the process of adding powdered dry peat to the wet peat from the bog, nor the addition of slaked lime thereto without the addition of pitch or its 95 equivalent to cause the peat fuel to burn with a luminous flame; but make reference to my pending applications filed May 27, 1919, Serial No. 300,123, and filed February 5, 1920, Serial No. 356,392, and filed December 2, 1920, Serial No. 427,852, which set forth and claim these features.

What I claim and desire to secure by Letters Patent is:—

1. The process of preparing fuel from 105 peat, which consists in stirring wet peat as obtained directly from the bog into an approximately putty-like consistency, gradually adding powdered pitch and powdered dry peat thereto, during the continuance of 110 the said treatment, continuing the stirring treatment until the three materials are

blended together to form a homogeneous mass, and pressing the same into blocks.

2. The process of preparing fuel from peat, which consists in stirring wet peat as obtained directly from the bog into an approximately putty-like consistency, gradually adding thereto, during the continuance of said treatment, enough powdered pitch to give a luminous flame, and enough powdered dry peat to give coherence without excess of moisture, continuing the treatment until the

materials are blended together to form a homogeneous mass, and pressing the mass into blocks.

In witness whereof I have hereunto signed my name in the presence of two subscribing witnesses.

SAMUEL CLELAND DAVIDSON.

Witnesses:

ALFRED AGAR,  
GERARD W. MATTHEW.